

1

3,275,668

**ORGANOMETALLIC ORTHOPHOSPHATES**  
 Anthony J. Revukas, Cranford, N.J., assignor to Cities  
 Service Oil Company, a corporation of Delaware  
 No Drawing. Filed July 31, 1961, Ser. No. 127,840  
 8 Claims. (Cl. 260—429.3)

This application is a continuation-in-part of my application S.N. 27,294, filed on May 6, 1960, now abandoned.

This invention relates to novel metallic orthophosphate compounds and to gasoline compositions including such compounds.

The use of lead compounds to increase the octane rating of gasoline is extremely common. Unfortunately, the addition of lead, while substantially increasing the octane ratings of gasolines to which it is added, at the same time has several drawbacks. Of these drawbacks the most serious is probably the tendency of the lead to increase undesirable surface ignition in the combustion chambers of the internal combustion engines in which the leaded gasoline is used. It has been the practice previously to utilize various phosphorous compounds in an attempt to reduce or prevent such surface ignition, but the use of such compounds has generally led to additional difficulties such as lead deposits on cylinder heads and valves.

It is an object of the present invention to provide novel metallic orthophosphate compounds adapted for use in improved gasoline compositions.

It is another object of the invention to provide an improved gasoline composition especially adapted to resist surface ignition.

The novel compounds of the present invention are orthophosphates of titanium or zirconium. Preferred orthophosphates of these metals may be represented by the general formula



wherein M represents zirconium or titanium, X is a number equal to the valence of the metal M and R and R' each represent a hydrocarbon radical having from 2 to 30 carbon atoms. In such compounds titanium and zirconium each have a valence of either 3 or 4 depending upon the starting material used. Preparation of these compounds is discussed in greater detail below. R and R' may represent identical or different hydrocarbon radicals. While any hydrocarbon radicals having between 2 and about 30 carbon atoms and soluble to the required extent in gasoline may be used, at least one of R and R' preferably represents a branched chain hydrocarbon radical. Such radicals are generally more soluble in gasoline than other hydrocarbon radicals, thereby facilitating the use of the novel compounds of the present invention as gasoline additives. Since chains of more than about 30 carbon atoms are generally difficult or impossible to dissolve in gasoline compositions, it is preferred that the hydrocarbon radicals of the orthophosphates of the present invention each have been 2 and about 30 carbon atoms.

Compounds of the present invention having branched chain alkyl hydrocarbon radicals include for instance the following:

titanium tetra (bis(2-methylpropyl) orthophosphate)  
 zirconium tetra (bis(3-butylloctyl) orthophosphate)  
 titanium tetra (bis(5-pentylhexadecyl) orthophosphate)  
 titanium tetra (bis(2-ethyl-5-butyltridecyl) orthophosphate)  
 zirconium tetra (bis(2-propyldecel) orthophosphate)  
 titanium tetra (bis(2,4-diethyloctyl) orthophosphate)  
 titanium tetra (bis(2-methyloctyl) orthophosphate)

2

zirconium tetra (bis(methylethyl) orthophosphate)  
 titanium IV di(2-ethylhexyl), tributyl orthophosphate  
 titanium tetra (bis(methylethyl) orthophosphate)  
 titanium tetra (2-methylpropyl, methylethyl

orthophosphate)  
 titanium tetra (2-methyloctyl, 2-propyldecel  
 orthophosphate)  
 titanium IV di(2-ethylhexyl), di(methylethyl), di(2-  
 methylpropyl), di(3-butylloctosyl) orthophosphate  
 titanium tri (bis(2-ethylhexyl) orthophosphate)  
 zirconium tetra (bis(2-ethylhexyl) orthophosphate)  
 zirconium tri (2-ethylhexyl, 2-methylpropyl  
 orthophosphate)

Compounds of the present invention having alkylaryl hydrocarbon radicals include for instance, the following:

titanium tetra (bis(octylphenyl) orthophosphate)  
 zirconium tetra (bis(methylphenyl) orthophosphate)  
 titanium tetra (bis(tricosylphenyl) orthophosphate)  
 zirconium tetra (bis(pentylphenyl) orthophosphate)  
 titanium tetra (octylphenyl, pentylphenyl  
 orthophosphate)  
 titanium tri (bis(methylphenyl) orthophosphate)  
 zirconium tri (bis(hexylphenyl) orthophosphate)

Compounds of the present invention having both alkyl and alkylaryl hydrocarbon radicals include, for instance, the following:

zirconium tetra (2-ethylhexyl, methylphenyl)  
 orthophosphate  
 titanium IV di(2-ethylhexyl), di(octylphenyl), 2-  
 propyldecel, methylethyl, di(2-methyloctyl)  
 orthophosphate

Compounds of the present invention having straight chain hydrocarbon radicals include for instance the following:

zirconium tetra (bis(octyl) orthophosphate)  
 titanium tetra (bis(ethyl) orthophosphate)  
 titanium tetra (methyldecel orthophosphate)  
 zirconium IV dibutyl, dihexyl, ethylhexyl, dipentyl  
 orthophosphate  
 titanium tetra (octylphenyl, hexyl orthophosphate)  
 zirconium tetra (2-ethylhexyl, butyl orthophosphate)  
 zirconium tetra (pentacosyl, hexadecyl orthophosphate)  
 titanium tri (bis(ethyl) orthophosphate)  
 zirconium tri (2-ethylhexyl, butyl orthophosphate)

The novel compounds described above are especially useful as gasoline additives in forming novel gasoline compositions adapted to resist surface ignition. In addition to resisting surface ignition, these additives generally inhibit rust and carburetor icing. In accordance with a preferred embodiment of the present invention a gasoline composition is provided which comprises a major proportion of a leaded hydrocarbon base fuel boiling in the gasoline range and containing between about 0.001 and about 5.0 theories of a titanium or zirconium orthophosphate. Such metallic orthophosphate preferably is of the type described above having the general formula



By the term "leaded gasoline," "leaded hydrocarbon base fuel boiling in the gasoline range" and similar terms is meant a petroleum fraction boiling in the gasoline boiling range (e.g., between about 50° and about 450° F.) to which has been added a small amount, such as between about 0.1 and about 6.0 cc. per gallon, of a metallo-organic antiknock compound such as tetraethyl lead (TEL), tetramethyl lead (TML), tetraisopropyl lead, etc. Lead is frequently present in gasoline compositions of

the present invention in the form of TEL, TML or mixtures of the same which may be present in suitable amounts such as between about 0.1 and about 6.0 cc. per gallon of gasoline composition, more usually between about 0.5 and about 4.0 cc. per gallon.

The novel metallic orthophosphates described above for use in leaded gasoline compositions in accordance with the present invention are present in suitable amounts such as between about 0.001 and about 5.0 theories, preferably between about 0.02 and about 2.0 theories. The term "theory" is intended in this context to designate the amount of additive required for the metal in the additive to react stoichiometrically with the lead in the compound such as TEL to produce the appropriate compound such as lead metatitanate.

In addition to the above described titanium and lead compounds, gasoline compositions contemplated by the present invention may include one or more other ingredients such as lead scavengers, gum inhibitors, lubricants, rust inhibitors, metal deactivators or other special purpose additives.

Lubricants suitable for use in the above described gasoline compositions may include, for instance, light hydrocarbon lubricating oils having viscosities at 100° F. of between about 50 and about 200 Saybolt Universal seconds (SUS) and viscosity indexes (VI) of between about 30 and about 120 with oil having a viscosity of about 100 SUS being preferred. Such oils may be present in suitable amounts such as between about 0.1 and about 1.0 volume percent of the gasoline composition.

When using lead compounds such as TEL, it is frequently found desirable to include with the lead a suitable lead scavenger for reducing the deposit of lead compounds within the combustion chamber. Such lead scavengers include for example halo hydrocarbon compositions such as ethylene dibromide and ethylene dichloride.

Gum inhibitors suitable for use in the above described gasoline compositions include conventional gum inhibitors such as 2,6-ditertiary-butyl para cresol. Such gum inhibitors may be present in suitable amounts such as between about 0.001 and about 0.006 volume percent of the gasoline composition. Likewise, a suitable metal deactivator is for example N,N'-disalicylidene-1,2-diaminopropane.

An especially valuable titanium compound of the type described above for use in gasoline compositions of the type described above is titanium tetra (bis(2-ethylhexyl) orthophosphate) having the formula



and hereinafter referred to as TIP.

Gasoline compositions of the present invention may be illustrated by the following examples. In most of these examples the gasoline compositions of the present invention are described as containing TIP. While TIP and the corresponding zirconium compound are preferred additives for use in such gasoline compositions, it should be understood that any of the other novel additive compounds contemplated by the invention, such as those described above, may be used in such gasoline compositions in place of or in addition to the TIP.

#### Example 1

A gasoline composition having excellent surface ignition characteristics may be prepared by adding the following ingredients to a suitable base gasoline:

TEL—2.2 cc. per gallon  
TIP—0.05 theory

The base gasoline used in blending this and other gasoline compositions of the invention may be a gasoline having the following characteristics:

|    | Distillation:           | ° F. |
|----|-------------------------|------|
|    | I.B.P. -----            | 101  |
| 5  | 10% evaporation -----   | 130  |
|    | 20% -----               | 149  |
|    | 30% -----               | 168  |
|    | 50% -----               | 210  |
|    | 70% -----               | 260  |
|    | 90% -----               | 328  |
|    | End point -----         | 409  |
| 10 | Recovery, percent ----- | 98.5 |
|    | Residue, percent -----  | 1    |
|    | Gravity, ° API -----    | 58.2 |

#### Example 2

Another suitable gasoline composition is prepared by adding the following ingredients to a suitable base gasoline:

TEL—2.2 cc. per gallon  
TIP—0.1 theory

#### Example 3

Another suitable gasoline composition is prepared by adding the following ingredients to a suitable base gasoline:

TEL—0.5 cc. per gallon  
TIP—0.25 theory

#### Example 4

Another suitable gasoline composition is prepared by adding the following ingredients to a suitable base gasoline:

TEL—4.0 cc. per gallon  
TIP—0.5 theory

Lubricating oil 1.0 volume percent (100 SUS, 95 VI)

#### Example 5

Another suitable gasoline composition is prepared by adding the following ingredients to a suitable base gasoline:

TEL—6.0 cc. per gallon  
TIP—5.0 theory

#### Example 6

Another suitable gasoline composition is prepared by adding the following ingredients to a suitable base gasoline:

TEL—0.1 cc. per gallon  
TIP—0.005 theory

#### Example 7

Another suitable gasoline composition is prepared by adding the following ingredients to a suitable base gasoline:

TEL—1.5 cc. per gallon  
TIP—0.01 theory  
Lubricating oil 0.1 volume percent (100 SUS, 95 VI)

#### Example 8

Another suitable gasoline composition is prepared by adding the following ingredients to a suitable base gasoline:

TEL—3.0 cc. per gallon  
Zirconium tetra bis(octylphenyl)orthophosphate—  
2.0 theory

#### Example 9

Another suitable gasoline composition is prepared by adding the following ingredients to a suitable base gasoline:

TEL—2.0 cc. per gallon  
Titanium tetra bis(octylphenyl)orthophosphate—  
0.5 theory

## Example 10

Another suitable gasoline composition is prepared by adding the following ingredients to a suitable base gasoline:

TEL—2.2 cc. per gallon

TIP—0.1 theory

Lubricating oil 0.25 volume percent (100 SUS, 95 VI)

Novel additive compounds of the type described above may be prepared in any suitable manner. According to one method of preparation, a suitable organic hydrogen phosphate or a mixture of such phosphates is placed in a reaction flask together with about half its volume of a suitable solvent such as dry toluene. The reaction flask is preferably equipped with a mechanical stirrer, thermometer, gas inlet tube, reflux condenser and a pressure equalizing funnel with its long stem dipping into the solution. The temperature in the reaction flask is raised to between about 110 and about 130° C. while stirring vigorously and titanium or zirconium tetrachloride with an equal volume of the solvent is added in spurts by means of the pressure equalizing delivery funnel. The tetrachloride is preferably introduced in amounts of about 1.1 moles of tetrachloride for each 4 moles of the organic hydrogen phosphate. Hydrogen chloride is evolved copiously by the reaction. Stirring and heating under reflux to 130° C. is continued until evolution of hydrogen chloride stops. Removal of by product hydrogen chloride is promoted by flushing the reaction flask with dry nitrogen by means of the gas inlet tube. The solvent is removed by distillation at reduced pressure such as 10 to 80 millimeters, the final temperature being about 130° C. The yield of product is usually between about 85 and about 95% of theory based on hydrogen phosphate.

In compounds prepared as described immediately above, the titanium or zirconium has a valence of 4. Similar compounds in which these metals have a valence of 3 may be prepared in a similar manner, e.g., by using titanium or zirconium trichloride rather than tetrachloride as a starting material.

## Example 11

In the production of TIP by means of the above procedure 2000 grams of commercial di(2-ethylhexyl) hydrogen phosphate (6 moles) and 330 grams (1.7 moles) of titanium tetrachloride were brought into reaction. The resulting solvent-free crude product was washed with water to remove acidic materials, taken up in half its volume of normal pentane, and dried over anhydrous sodium sulfate. After filtering, the pentane was removed by distillation with the final temperature being 130° C. at 20 millimeters pressure. The yield of dark, amber colored liquid TIP was 1900 grams or 95% of theory based on acid phosphate. Percentages of titanium and phosphorous obtained on analysis were as follows:

Theory: Titanium, 3.59%; phosphorous, 9.29%. Actually found: Titanium, 3.70%; phosphorous, 8.94%.

This TIP had a viscosity at 100° F. of 1337 SUS and at 210° F. of 180 SUS. The density of this TIP at 20° C. was 1.055.

In forming the TIP as described above the reaction is formulated as follows:



## Example 12

In order to demonstrate the usefulness of novel compounds of the type described above which include alkyl-aryl radicals as gasoline additives, titanium tetra (bis-

(octylphenyl) orthophosphate) was prepared in accordance with the general method of preparation described above. This compound was solid but was moderately soluble in gasoline and is, therefore, suitable as a gasoline additive.

## Example 13

Another titanium orthophosphate containing branched chain hydrocarbon radicals was prepared by reacting 0.2 mole each of monobutyl hydrogen phosphate, dibutyl hydrogen phosphate and di(2-ethylhexyl) hydrogen phosphate with 0.22 mole titanium tetrachloride in the manner described above. A 92% yield based on titanium tetrachloride was obtained of titanium IV di(2-ethylhexyl)-tributyl orthophosphate having the formula:



This compound was a resinous amber colored solid which was soluble in gasoline. An analysis for titanium yielded the following results:

Theory: 6.56%. Actually found: 6.55%.

## Example 14

Zirconium orthophosphate was prepared according to the general procedure described above by reacting 0.11 mole of zirconium tetrachloride with 0.40 mole of di(2-ethylhexyl) hydrogen phosphate in the presence of 300 milliliters of toluene. The product was zirconium tetra (bis (2-ethylhexyl) orthophosphate) having the formula:



In order to evaluate the characteristics of gasoline compositions of the present invention, three separate gasoline compositions (A, B, and C) were prepared. These gasoline compositions contained metallic orthophosphate additives of the present invention as indicated in Tables I and II below.

Gasoline compositions A and B used the base gasoline described above in connection with Example 1 with 2.2 cc. per gallon of TEL added. Gasoline composition C also used a base gasoline having the same properties as the base gasoline of Example 1. The base gasoline of Example C also contained 2.2 cc. per gallon of TEL but had been stored for a shorter period of time prior to the tests described below than had the base gasolines of gasoline compositions A and B. The base gasolines of gasoline compositions B and C also contained 0.25 volume per percent of 100 SUS (95 VI) light lubricating oil. The base gasolines of gasoline compositions A, B and C thus differed from the compositions A, B and C respectively only in the presence or absence of the metallic orthophosphate additives of the present invention. The gasoline compositions A, B and C, as well as their respective base gasolines were subjected to both single cylinder and multi-cylinder engine deposit tests as described below.

The single cylinder engine deposit tests were run in CFR engines having L head assemblies and compression ratios of 7 to 1. Each test consisted of alternating periods of operation under idling conditions for 50 seconds followed by operation under full load conditions for 150 seconds. These cycles were continued for a total test time of at least 40 hours for each test. During these tests the engine air intake temperature was maintained at 115° F. while the oil temperature was maintained at 160° F. and the coolant temperature at 150° F. During the idling portions of the tests the engines were operated with an air to fuel ratio of 12 to 1 at 600 r.p.m. while during

the full load portions of the tests the engines were operated with air to fuel ratios of 13 to 1 and at 900 r.p.m. During the test, the number of wild pings (indicating pre-ignition) was counted by an Erwin Instrument Co. Wild

dicates clearly that the addition of the zirconium or titanium orthophosphate substantially reduced the octane number increases due to engine deposits as well as the LIB requirements. For instance, with TIP in the gaso-

TABLE II.—MULTICYLINDER ENGINE DEPOSIT TEST

| Gasolene Composition | Orthophosphate Additive                              | Theories of Additive | Octane Requirement Increase (ORI) Base Gasolene |               | LIB Requirements Base Gasolene |               |
|----------------------|------------------------------------------------------|----------------------|-------------------------------------------------|---------------|--------------------------------|---------------|
|                      |                                                      |                      | Without additive                                | With additive | Without additive               | With additive |
| A-----               | TIP-----                                             | 0.05                 | 14.5                                            | 5.5           | 85                             | 55            |
| B-----               | TIP-----                                             | 0.10                 | 14.5                                            | 4.5           |                                |               |
| C-----               | Zirconium tetra (bis (2-ethylhexyl) orthophosphate). | 0.20                 | 24.8                                            | 5.2           | 100+                           | 60            |

Ping Counter. At the end of the test the average of the wild pings per hour was determined by plotting the total wild pings versus time and taking the slope of the curve. This measurement served as a reliable indication of the surface ignition characteristics of the fuel being tested.

The multi-cylinder engine deposit tests were run in 1958 Oldsmobile Rocket engines having compression ratios of 10 to 1. The total time of each of these tests was 120 hours of operation in cycles of 50 seconds operation under idling conditions followed by 150 seconds operation under load conditions to develop twelve brake horsepower. During the idle portions of the cycle the engines were operated with an air to fuel ratio of 12 to 1 at a speed of 600 r.p.m. and with a coolant temperature of 160° F. During the load portions of the test the engines were operated with an air to fuel ratio of 14 to 1 at 2000 r.p.m. and with a coolant temperature of 160° F. Oil temperature was not controlled during these tests. At intervals of 16 to 24 hours the octane requirement increase (ORI) was obtained by full throttle operation at 1000 r.p.m. using primary reference fuels and varying spark advance for trace knock. At the end of the test the LIB requirement (leaded iso-octane-benzene reference fuel with 3 cc. per gallon TEL to yield trace rumble) was obtained. The LIB requirement was obtained at 1500 r.p.m. and was the LIB fuel needed to prevent rumble at wide open throttle.

The results of the single cylinder engine deposit test on the gasolene compositions A, B and C and their respective base gasolenes described above are given in Table I below while the results of the multicylinder engine deposit tests are given in Table II.

TABLE I.—SINGLE CYLINDER ENGINE DEPOSIT TEST

| Gasolene Composition | Orthophosphate Additive                              | Theories of Additive | Average Wild Pings Per Hour Base Gasolene |               | 65 |
|----------------------|------------------------------------------------------|----------------------|-------------------------------------------|---------------|----|
|                      |                                                      |                      | Without additive                          | With additive |    |
| A-----               | TIP-----                                             | 0.05                 | 25                                        | 2             |    |
| B-----               | TIP-----                                             | 0.10                 | 25                                        | 4             |    |
| C-----               | Zirconium tetra (bis (2-ethylhexyl) orthophosphate). | 0.20                 | 7                                         | <1            |    |

Table I shows clearly that the addition to the titanium or zirconium orthophosphate to the base gasolene resulted in gasolene compositions having remarkably good surface ignition characteristics as evidenced by a decrease in wild pings as compared with the base gasolene which did not contain these additives. Likewise, Table II in-

25 lene the Oldsmobile engines tolerated a three times greater amount of the surface ignition inducing aromatic benzene than did the base gasoline, thereby further attesting to the high surface ignition resistance quality of the gasoline compositions containing the metallic orthophosphates of the present invention.

In order to evaluate the ability of TIP to inhibit carburetor icing, carburetor icing tests were conducted in a 30 standard six cylinder Chevrolet engine having a displacement of 216.5 cubic inches and rated at 86 horsepower at 3400 r.p.m. The following test conditions were employed.

- 35 Intake air 38 to 40° F.  
 Relative humidity 100%  
 Engine load 10 horsepower  
 Engine speed 1500 r.p.m.  
 Idle speed 450 to 500 r.p.m.  
 40 Temperature of fuel entering carburetor 48 to 50 F.  
 Air to fuel ratio 12.3 to 12.5

45 Carburetor icing tendencies of gasolines are measured by this test when the engine is operated under the constant severe icing conditions outlined above. The engine run is started with the throttle plate at 34° F. The ice forming characteristics of the test gasoline normally control the engine operating cycle. During the test the engine is run at 1500 r.p.m. for 1 to 2½ minutes. At the end of the 1500 r.p.m. operating cycle the throttle is returned to the idle speed of 450 to 500 r.p.m. The engine is idled for 30 seconds and if stalling does not occur the idle speed r.p.m. is observed. A reduction in idle speed of more than 100 r.p.m. is considered a partial stall.

50 The base gasoline used in the carburetor icing tests had the following volatility characteristics:

|                           |         |      |
|---------------------------|---------|------|
| Gravity -----             | ° API   | 60.0 |
| Reid vapor pressure ----- | lbs.    | 10.9 |
| ASTM distillation:        |         |      |
| 60 I.B.P. -----           | ° F.    | 81   |
| 5% evaporated @ -----     | ° F.    | 102  |
| 10 -----                  | ° F.    | 112  |
| 30 -----                  | ° F.    | 146  |
| 50 -----                  | ° F.    | 188  |
| 70 -----                  | ° F.    | 250  |
| 90 -----                  | ° F.    | 315  |
| 95 -----                  | ° F.    | 335  |
| E.P. -----                | ° F.    | 359  |
| Recovery -----            | percent | 97.4 |
| Residue -----             | percent | 1.1  |
| Loss -----                | percent | 1.5  |

70 75 A total of 12 test runs were made. In four of these runs the base gasoline contained no additive except 2.2 cc. per gallon TEL. In another series of four runs the base gasoline used contained 0.024 theory TIP while in the

remaining four runs the base gasolene contained 0.096 theory TIP. The results of these carburetor icing tests are shown in Table III below.

TABLE III.—STALLING CHARACTERISTICS OF GASOLENE WITH AND WITHOUT TIP

| Operating Time at Idle<br>(min.) | Amount of TIP in Base Gasolene<br>(theories) |       |       |
|----------------------------------|----------------------------------------------|-------|-------|
|                                  | 0                                            | 0.024 | 0.096 |
| 0.5                              | S                                            | ----- | ----- |
| 1.0                              | S, S, S                                      | N     | ----- |
| 2.5                              | -----                                        | ----- | ----- |
| 3.0                              | -----                                        | N, N  | ----- |
| 3.5                              | -----                                        | ----- | N, N  |

S indicates stalling occurred.

N indicates no stalling occurred.

The results show clearly that when TIP was not used the engine stalled within  $\frac{1}{2}$  to 1 minute after the throttle was returned to the idle position. Stalling is attributable to ice formation around the periphery of the throttle plate when it was nearly closed at idle. During these runs the ice was observed to build up, particularly in the throttle plate swivel area, thereby restricting the air flow. Such icing is especially prevalent in the wintertime because the more volatile winter grade gasolines aggravate icing tendencies due to their greater tendency to evaporate with resulting cooling. Also, weather conditions frequently introduce enough moisture to create icing problems when relative humidity of the atmosphere is above about 85% and the temperature between about 35 and about 47° F. In contrast to the poor stalling characteristics displayed by the base gasolene under the test conditions described above, the gasolene containing TIP prevented ice build up in the throttle plate zone as observed visually during the test and also as demonstrated by the absence of stalling during  $3\frac{1}{2}$  minutes of engine operation with the throttle in idle position during the above described test. It is, therefore, apparent that the addition of TIP to the base gasolene served to eliminate the stalling tendencies of the base gasolene. TIP is thus shown to be a superior gasolene additive in that it not only reduced preignition problems as described above, but also reduces or eliminates carburetor icing and prevents rusting as determined by ASTM Method D665-54 Test for Rust-Preventing Characteristics of Oil, when performed at ambient temperature.

While the invention has been described above with respect to certain preferred embodiments thereof, it will be understood by those skilled in the art that various changes

and modifications may be made without departing from the spirit and scope of the invention and it is intended to cover all such changes and modifications in the appended claims.

5 I claim:

1. A liquid compound having the formula:



10 wherein M is a metal selected from the group consisting of titanium and zirconium and each of R and R' is a branched chain alkyl having up to about 30 carbon atoms.

2. A liquid compound having the formula:



20 wherein M is a metal selected from the group consisting of titanium and zirconium, X is a number equal to the valence of the metal M and each of R and R' is a branched chain alkyl having up to about 30 carbon atoms.

25 3. A compound of claim 2 in which R and R' are identical branched chain alkyls.

4. Titanium tetra (bis(2-ethylhexyl) orthophosphate).

5. Zirconium tetra (bis(2-ethylhexyl) orthophosphate).

6. Titanium tri (bis(2-ethylhexyl) orthophosphate).

7. Zirconium tri (bis(2-ethylhexyl) orthophosphate).

30 8. A compound of claim 1 wherein the metal is titanium.

#### References Cited by the Examiner

##### UNITED STATES PATENTS

|    |           |         |                                 |
|----|-----------|---------|---------------------------------|
| 35 | 2,228,659 | 1/1941  | Farrington et al. ----- 252—35  |
|    | 2,346,155 | 4/1944  | Denison et al. ----- 252—32     |
|    | 2,480,673 | 8/1949  | Reiff et al. ----- 260—429.5 XR |
|    | 2,881,062 | 4/1959  | Bishop ----- 44—69              |
| 40 | 2,885,417 | 5/1959  | Heyden ----- 260—429.5 XR       |
|    | 2,913,469 | 11/1959 | Russell ----- 260—429.5         |
|    | 2,926,183 | 2/1960  | Russell ----- 260—429.5         |
|    | 2,948,599 | 8/1960  | Orloff et al. ----- 44—69       |
|    | 3,055,925 | 9/1962  | Hartle ----- 260—437            |

45 45 TOBIAS E. LEVOW, Primary Examiner.

JULIUS GREENWALD, ABRAHAM H. WINKELSTEIN, Examiners.

50 M. WEINBLATT, W. J. VAN BALEN, H. M. S. SNEED, Assistant Examiners.

UNITED STATES PATENT OFFICE  
CERTIFICATE OF CORRECTION

Patent No. 3,275,668

September 27, 1966

Anthony J. Revukas

It is hereby certified that error appears in the above numbered patent requiring correction and that the said Letters Patent should read as corrected below.

Column 4, line 74, for "(octylphenylorthophosphate-" read  
-- (octylphenyl)orthophosphate --; column 5, lines 67 to 70, the  
formula should appear as shown below instead of as in the patent:



Column 6, line 15, the formula should appear as shown below  
instead of as in the patent:



Signed and sealed this 29th day of August 1967.

(SEAL)  
Attest:

ERNEST W. SWIDER  
Attesting Officer

EDWARD J. BRENNER  
Commissioner of Patents